

## UNITED STATES PATENT OFFICE

2,205,876

## BEARING

William J. Conley, Rochester, N. Y., assignor to  
 E. Phelps Langworthy, Rochester, N. Y.

No Drawing. Application September 9, 1937,  
 Serial No. 163,059

7 Claims. (Cl. 308—242)

This invention relates to improvements in bearings.

Standard bearings are, for the most part, produced from alloys, the different metals of which provide hard and soft constituents. The former have a relatively low coefficient of friction and are adapted to carry the load while the latter provide a plastic bed or matrix in which the harder constituents are permitted to adjust 5 themselves to accommodate the journal or other part through which the load is transmitted to the bearing. In order to insure satisfactory performance it is essential that the hard constituents be present in an amount which will enable them 10 to carry the entire load applied to the bearing without becoming dislodged or wearing excessively, the proportions of the metals being predetermined with this object in view. A bearing of the character described, however, has the objection 15 that it has a different coefficient of expansion from the part through which the load is transmitted to it. Hence when the said part is a journal, for example, the clearance between it and the bearing varies as the working temperature varies, thereby preventing the said parts from being fitted in such a manner that a proper clearance will be maintained at all temperatures. Such a bearing has the further objection 20 that it is of low strength and must, therefore, in installations in which a high strength characteristic is required be employed as a lining for a brass or holder of a stronger metal.

The principal object of the present invention is to overcome the above objections, this object 25 contemplating the use of spheroidized steel for both the bearing and the journal or other part through which the load is transmitted to the bearing and involving the adjustment of the micro-structures of the co-operating parts to prevent excessive abrasion, galling or any other disturbance of the surfaces which would precede 30 wearing or scoring of the contacting surfaces.

A further object is to provide a bearing having the same coefficient of expansion as the part 35 through which the load is transmitted to it.

A still further object is to provide a bearing of high strength.

A still further object is to provide for simplicity and economy in the manufacture and assembly of the bearing and cooperating part.

In the practice of the invention a steel having a carbon content in excess of .3% is preferably employed. Such a steel consists of laminated zones of cementite and ferrite surrounded by a 50 network of ferrite if the carbon content is sub-

stantially less than .8% and a network of cementite if the carbon content is substantially in excess of this amount. The steel described is spheroidized in any suitable manner. It may, for example, be initially heated to a temperature 5 of the order of 1500° F. to cause the cementite to enter into solution with the ferrite and then quenched and reheated to a temperature in the range of 1100° F.—1400° F. to cause the formation of globular cementite. The steel is held at this 10 latter temperature until a predetermined cementite count is obtained, the cementite particles thus produced being uniformly distributed throughout the matrix or bed provided by the ferrite.

I have discovered that, when the heat treatments referred to are so regulated as to produce a cementite count in a range centering about  $28 \times 10^7$  spheroids per square inch and the steel thus produced is employed to produce a bearing 20 and the journal or other part through which the load is transmitted to the bearing, dry contacting surfaces are provided which have a coefficient of friction comparing favorably to that of bronze on steel, i. e. between .30 and .40, and hence 25 which will prevent excess wearing or scoring if for any reason the parts are not properly lubricated. The cementite particles in the bearing carry the load while the ferrite particles provide 30 for their adjustment. In this respect, therefore, 35 the constituents of the bearing function in substantially the same manner as those of an alloy bearing. It will be noted, however, that in the present instance the journal or other part through which the load is transmitted to the bearing has a structure similar to that of the bearing, i. e., hard and soft constituents of cementite and ferrite, respectively, and that the said constituents have the same functions as those of the bearing. In other words both the 40 bearing and the part through which the load is transmitted to the bearing are structurally similar and provision is made for the automatic adjustment of the load supporting constituents of each.

It is to be noted that not only must the bearing and journal or other part be similar in structure and have substantially the same cementite count in order to prevent excess wearing or scoring in the absence of a lubricating medium but the cementite count itself must be within a predetermined range. The count of  $28 \times 10^7$  above noted is substantially the value at which optimum results can be obtained. When a steel having a carbon content of .8% was employed the average 55

area of the cementite particles was found to be of the order of  $.64 \times 10^{-9}$ . As steels of a lower cementite count are employed wearing and scoring of the contacting surfaces increase progressively 5 until at a count of the order of  $17 \times 10^7$  no practical results can be obtained. In a like manner wearing and scoring of the contacting surfaces increase progressively as the cementite count is raised beyond  $28 \times 10^7$ , although not so rapidly as 10 when the count is reduced. A steel having a count of  $40 \times 10^7$ , for example, has proved to be partially satisfactory as will, no doubt, steels having a higher count.

From the foregoing it will be apparent that the 15 use of spheroidized steel in the manner described has the advantage that it enables a bearing to be produced from the same metal as the journal or other part through which the load is transmitted to the bearing. The bearing and journal or other 20 part thus have the same coefficient of expansion and can, therefore, be fitted so that the desired clearance will be maintained under varying operating temperatures. The use of spheroidized steel has the further advantages that it enables 25 the production of bearings stronger than those of alloys and provides for facility and economy in the manufacture and assembly of the parts.

I claim as my invention:

1. A bearing assembly comprising companion 30 relatively movable parts which are formed to provide cooperating contacting surfaces, said parts being of spheroidized steel and having cementite counts at said surfaces which are substantially equal and which are in excess of  $17 \times 10^7$  and less 35 than  $28 \times 10^7$  spheroids per square inch.

2. A bearing assembly comprising companion 40 relatively movable parts which are formed to provide cooperating contacting surfaces, said parts being of spheroidized steel and having cementite counts at said surfaces which are substantially equal and in excess of  $17 \times 10^7$  spheroids per 45 square inch.

3. A bearing assembly comprising companion 45 relatively movable parts which are formed to provide cooperating contacting surfaces, said parts being of spheroidized steel and having cementite counts at said surfaces which are substantially equal and whereby easily machined cooperating

steel bearing surfaces are provided being substantially equal in respect to coefficient of expansion, friction, hardness, and resistance to surface disturbance in a range centering about  $28 \times 10^7$  spheroids per square inch.

4. The method of manufacturing mating steel bearing surfaces comprising spheroidizing the steel to be used so that the mating surfaces comprise spheroidized steel having spheroid carbide counts which are substantially equal and which are of a size ranging from approximately  $17 \times 10^7$  to  $28 \times 10^7$  spheroids per square inch whereby easily machined steel bearing surfaces are provided being substantially equal in respect to coefficient of expansion, friction, hardness, and resistance to surface disturbance.

5. A bearing, the component parts of which comprise metals having a high melting point, said parts being formed of spheroidized steel, the carbide counts thereof ranging above  $17 \times 10^7$  20 spheroids per square inch whereby close fitting, high-heat-resisting bearing parts may be provided moving relatively with the minimum of mechanical interference between the respective spheroids of said parts with and without lubricant 25 and in temperatures up to the range where said carbide particles are disintegrated, or caused to change their form.

6. A bearing metal comprising an easily machinable ferritic mass having heterogeneously arranged therein a plurality of hard globular carbide particles and being of a size and number ranging above  $17 \times 10^7$  globules per square inch whereby a mass of similar hardness in the absence of lubricant may easily move in bearing 35 relation thereto with a minimum of mechanical and frictional resistance.

7. A bearing comprising cooperating steel bearing members, each having a steel bearing surface movable and in contact relatively to each other, composed of spheroidized steel, the spheroid counts thereof ranging above  $17 \times 10^7$  globules per square inch whereby easily machined hard surfaced, long-life bearing members are obtained when machined, requiring no further heat treat- 45

WILLIAM J. CONLEY.